

## UNITED STATES PATENT OFFICE

HENRY DREYFUS, OF LONDON, GEORGE HOLLAND ELLIS, TOBIAS OCKMAN, AND HENRY CHARLES OLPIN, OF SPONDON, NEAR DERBY, ENGLAND, ASSIGNEES TO CELANESE CORPORATION OF AMERICA, A CORPORATION OF DELAWARE

DYEING, PRINTING, OR STENCILLING OF MATERIALS MADE OF OR CONTAINING CELLULOSE DERIVATIVES

No Drawing. Application filed April 19, 1929, Serial No. 356,300, and in Great Britain April 26, 1928.

This application, which is a continuation in part of U. S. application Serial No. 162,938 filed 22nd January 1927, relates to the dyeing, printing, stencilling or otherwise colouring of threads, yarns, knitted or woven fabrics or other products made of or containing cellulose acetate or other organic acid esters of cellulose, such for example as cellulose formate, propionate, or butyrate, or the products obtained by the treatment of alkalinized cellulose with esterifying agents (e. g. the product known as "immunized cotton"), or made of or containing cellulose ethers, such as methyl, ethyl, or benzyl cellulose, or the corresponding condensation products of cellulose and glycols or other polyhydric alcohols, all of which cellulose derivatives are hereinafter referred to as organic substitution derivatives of cellulose.

U. S. application Serial No. 162,938 describes and claims, inter alia, the dyeing or otherwise colouring of the said organic substitution derivatives of cellulose by means of dyestuffs or compounds containing one or more urea or thiourea residues. In the course of further researches it has been found that especially useful results are obtained by dyeing or otherwise colouring the cellulose acetate or other organic substitution derivatives of cellulose with particular unsulphonated colouring matters or compounds of this class which contain one urea or thiourea group in which one or more hydrogen atoms of the said group is or are replaced by aryl groups, at least one of which contains one or more nitro groups. The aryl groups may contain further substituents such as halogen, or alkyl, alkyloxy, amino, or acidylamino groups. When the colouring matters contain diazotizable amino groups they may be diazotized on the materials and developed in the customary manner.

The following table shows the shades given

| Colouring matter                                                      | Shade         |
|-----------------------------------------------------------------------|---------------|
| 2: 4-dinitrophenylurea                                                | Yellow        |
| 2: 4: 2': 4'-tetranitro-diphenylurea                                  | Yellow        |
| Dinitrodiaminodiphenylurea from nitro-m-phenylenediamine and phosgene | Golden yellow |

The colouring matters or compounds may be applied in aqueous solution (when sufficiently soluble), or in aqueous suspensions or colloidal solutions or dispersions obtained by grinding (for example in colloid mills), by dissolving in a solvent and pouring into water containing or not containing protective colloids or dispersors, by pretreating the colouring matters or compounds with dispersing agents or by other methods. Of the dispersing agents which are suitable for obtaining such dispersions may be mentioned those described in U. S. Patent specifications Nos. 1,618,413, 1,618,414 and 1,694,413, and British Patents Nos. 273,819 and 273,820; viz. bodies of oily or fatty characteristics, namely higher fatty acids or sulphonated or other derivatives thereof containing salt-forming groups, such as sulphorcinoleic acid or other sulphonated fatty acids or salts of such acids or bodies, for instance their alkali or ammonium salts, used alone or in conjunction with auxiliary solvents as described in U. S. Patent specification No. 1,690,481 and British Patent No. 269,960; carbocyclic compounds containing in their structure one or more salt forming groups or salts of such compounds; sulpho-aromatic fatty acids or salts thereof; and soluble resin soaps or sodium or other soluble salts of resin acids.

Mixed goods containing for example, in addition to the organic substitution derivative or derivatives of cellulose, cotton, silk, wool, or the cellulose type of artificial silk or other fibres or threads, may be dyed or otherwise coloured with or without employment of

other dyestuffs or components according to the character of the threads or fibres used in association, such other dyestuffs or components being applied if desired either before or after the application of the colouring matters or compounds of the present invention, or when not deleteriously affected thereby, they may be applied in conjunction therewith.

The following example illustrates the invention but is not to be regarded as limiting it in any way.

*Example 1*

To dye a yellow shade on 10 kilos of cellulose acetate yarn in hank form, 100 grams of finely ground 2, 4-dinitro-phenylurea are well stirred or ground with 1 litre of sodium sulphuricinoleate (50%); the mixture is heated under an open steam pipe, and then diluted with boiling water, and further boiled. The liquor is then passed through a filter cloth into a dyebath containing 300 litres of cold soft water. 10 kilos of the material are introduced and dyeing is carried out as usual, the temperature being raised in  $\frac{3}{4}$  hour to 75-80° C. and maintained at this level as necessary to exhaust. The hanks are now lifted, rinsed, and dried, or otherwise treated as requisite.

By replacing the cellulose acetate yarn in this example by yarn made of cellulose formate the latter is likewise dyed in yellow shades.

What we claim and desire to secure by Letters Patent is:—

1. Process for dyeing materials comprising organic substitution derivatives of cellulose which comprises applying thereto unsulphonated colouring matters of the general formula



where X represents oxygen or sulphur and  $R_1$ ,  $R_2$ ,  $R_3$ , and  $R_4$  represent hydrogen, or aryl residues but at least one is a nitroaryl residue.

2. Process for dyeing materials comprising organic substitution derivatives of cellulose which comprises applying thereto diazotizable unsulphonated colouring matters of the general formula



where X represents oxygen or sulphur and  $R_1$ ,  $R_2$ ,  $R_3$ , and  $R_4$  represent hydrogen, or aryl but at least one is a nitroaryl residue, and diazotizing and developing with an azo coupling component.

3. Process for dyeing materials comprising cellulose acetate which comprises applying

thereto unsulphonated colouring matters of the general formula



where X represents oxygen or sulphur and  $R_1$ ,  $R_2$ ,  $R_3$  and  $R_4$  represent hydrogen, or aryl residues but at least one is a nitroaryl residue.

4. Process for dyeing materials comprising cellulose acetate which comprises applying thereto diazotizable unsulphonated colouring matters of the general formula



where X represents oxygen or sulphur and  $R_1$ ,  $R_2$ ,  $R_3$ , and  $R_4$  represent hydrogen, or aryl residues but at least one is a nitroaryl residue, and diazotizing and developing with an azo coupling component.

5. Process for dyeing materials comprising cellulose acetate which comprises applying thereto in aqueous colloidal dispersion unsulphonated colouring matters of the general formula



where X represents oxygen or sulphur and  $R_1$ ,  $R_2$ ,  $R_3$ , and  $R_4$  represent hydrogen, or aryl residues but at least one is a nitroaryl residue.

6. Materials comprising organic substitution derivatives of cellulose dyed with unsulphonated colouring matters of the general formula



where X represents oxygen or sulphur and  $R_1$ ,  $R_2$ ,  $R_3$ , and  $R_4$  represent hydrogen, or aryl residues but at least one is a nitroaryl residue.

7. Materials comprising cellulose acetate dyed with unsulphonated colouring matters of the general formula



where X represents oxygen or sulphur and  $R_1$ ,  $R_2$ ,  $R_3$ , and  $R_4$  represent hydrogen, or aryl residues but at least one is a nitroaryl residue.

8. Process for dyeing materials comprising organic substitution derivatives of cellulose which comprises applying thereto un-

sulphonated colouring matters consisting of compounds of the formula:



5 where X represents oxygen or sulphur, substituted in at least one of the NH<sub>2</sub> groups by at least one nitroaryl residue.

9. Process for dyeing materials comprising cellulose acetate which comprises applying thereto unsulphonated colouring matters consisting of compounds of the formula:



15 where X represents oxygen or sulphur, substituted in at least one of the NH<sub>2</sub> groups by at least one nitroaryl residue.

10. Process for dyeing materials comprising organic substitution derivatives of cellulose which comprises applying thereto diazotizable unsulphonated colouring matters consisting of compounds of the formula:



25 where X represents oxygen or sulphur, substituted in at least one of the NH<sub>2</sub> groups by at least one nitroaryl residue and diazotizing and developing with an azo coupling component.

30 11. Process for dyeing materials comprising cellulose acetate which comprises applying thereto diazotizable unsulphonated colouring matters consisting of compounds of the formula:



where X represents oxygen or sulphur, substituted in at least one of the NH<sub>2</sub> groups by at least one nitroaryl residue and diazotizing and developing with an azo coupling component.

45 12. Process for dyeing materials comprising organic substitution derivatives of cellulose which comprises applying thereto unsulphonated colouring matters consisting of compounds of the formula:



50 where X represents oxygen or sulphur, substituted in at least one of the NH<sub>2</sub> groups by at least one nitrophenyl residue.

55 13. Process for dyeing materials comprising cellulose acetate which comprises applying thereto unsulphonated colouring matters consisting of compounds of the formula:



60 where X represents oxygen or sulphur, substituted in at least one of the NH<sub>2</sub> groups by at least one nitrophenyl residue.

65 14. Process for dyeing materials comprising organic substitution derivatives of cellulose which comprises applying thereto diazo-

tizable unsulphonated colouring matters consisting of compounds of the formula:



70 where X represents oxygen or sulphur, substituted in at least one of the NH<sub>2</sub> groups by at least one nitrophenyl residue and diazotizing and developing with an azo coupling component.

75 15. Process for dyeing materials comprising cellulose acetate which comprises applying thereto diazotizable unsulphonated colouring matters consisting of compounds of the formula:



80 where X represents oxygen or sulphur, substituted in at least one of the NH<sub>2</sub> groups by at least one nitrophenyl residue and diazotizing and developing with an azo coupling component.

85 16. Materials comprising organic substitution derivatives of cellulose dyed with unsulphonated colouring matters consisting of compounds of the formula:



90 where X is oxygen or sulphur, substituted in at least one of the NH<sub>2</sub> groups by at least one nitroaryl residue.

95 17. Materials comprising cellulose acetate dyed with unsulphonated colouring matters consisting of compounds of the formula:



100 where X is oxygen or sulphur, substituted in at least one of the NH<sub>2</sub> groups by at least one nitroaryl residue.

105 18. Materials comprising organic substitution derivatives of cellulose dyed with unsulphonated colouring matters consisting of compounds of the formula:



110 where X is oxygen or sulphur, substituted in at least one of the NH<sub>2</sub> groups by at least one nitrophenyl residue.

115 19. Materials comprising cellulose acetate dyed with unsulphonated colouring matters consisting of compounds of the formula:



120 where X is oxygen or sulphur, substituted in at least one of the NH<sub>2</sub> groups by at least one nitrophenyl residue.

125 In testimony whereof we have hereunto subscribed our names.

HENRY DREYFUS.  
GEORGE HOLLAND ELLIS.  
TOBIAS OCKMAN.  
HENRY CHARLES OLPIN.